

Dec. 18, 1956

H. A. SECRIST

2,774,128

FELT-LIKE PRODUCTS

Filed Nov. 4, 1950

*Fig. 1*



*Fig. 2*

INVENTOR.  
HORACE A. SECRIST.  
BY H. L. KIRKPATRICK  
ATTORNEY.

# United States Patent Office

2,774,128

Patented Dec. 18, 1956

1

2,774,128

## FELT-LIKE PRODUCTS

Horace A. Secrist, Dedham, Mass., assignor to The Kendall Company, Boston, Mass., a corporation of Massachusetts

Application November 4, 1950, Serial No. 194,195

1 Claim. (Cl. 28—79)

This invention relates to non-woven fabrics and felt-like sheet materials comprising interlocking cotton fibers and fibers having latent coalescent properties.

Many attempts have been made to manufacture non-woven fabrics by mixing cotton fibers and fusible fibers by some suitable means and thereafter activating the fusible fibers. Among the successful materials made in this manner is the fabric disclosed by Reed in U. S. Patent 2,277,049. According to the preferred process of Reed carded webs of intermingled cotton fibers and plasticized cellulose acetate fibers are unified by heat and pressure to form a fabric. Although this material and structures similar to it have enjoyed a wide variety of commercial uses, they still suffer from certain undesirable characteristics. The heat and pressure usually required to produce a strongly unified sheet material have caused the mixed fiber products of the prior art to lose thickness and have a somewhat harsh and papery feel. The primarily lengthwise alignment of fibers obtained by the carding or garneting process persists through to the finished product resulting in a highly directional fabric with a high ratio of lengthwise to widthwise strength, often of the order of 9 or 10 to 1. The extensibility is of the same order of magnitude as that of an untreated web or bat, namely 20 20% or less.

It is the primary object of this invention to provide a novel soft, porous, extensible felt-like sheet material having various advantages over the product just described and it is a special object of this invention to produce a reinforced cotton felt of high tensile strength in both the wet and dry states.

I accomplish these objects and others by supplying a sheet material comprising a network of intermingled cotton fibers and fibers having latent coalescent properties, the cotton fibers being frictionally entangled and interlocked with each other and with the fusible fibers in situ by artificially induced kinks, bends, twists and curls, and the fusible fibers being bonded to one another and/or the cotton fibers by coalescence. Depending upon the conditions of caustic treatment, the percentage of fusible fibers and the extent of activation thereof, the felt-like products of my invention may vary from soft, fluffy, absorbent, highly extensible materials to structures of limited extensibility and/or increased stiffness.

These and other characteristics of my invention will be more readily appreciated from the following description of an embodiment thereof selected for the purposes of illustration, and shown in the accompanying drawings in which:

Figure 1 is a plan view of a section of a fabric of my invention, and

Figure 2 is a cross section along line 2—2 of Figure 1.

As shown in these drawings, the fabric is made of a three-dimensional network consisting essentially of cotton fibers 10 which are frictionally interlocked and entangled with themselves and each other as a result of chemically induced random kinks, twists, bends and curls of said

2

cotton fibers, and coalescent fibers 12 which are commingled with the aforementioned cotton fibers, and which are adhesively bonded to some, at least, of the points of intersection of said coalescible fibers with each other and with the said cotton fibers.

The source of the integrity and coherence of my sheet materials is the frictional interlocking provided by the network of the curled and kinked cotton fibers, and the positive adhesive fiber-to-fiber bonding supplied by the fusible fibers which co-operate to give my products a combination of conformability, extensibility and strength. The adhesive bonds act as a framework permeating the structure, impeding and damping the inter-fiber adjustments which take place as my sheet materials are stressed. As the curled and kinked cotton fibers straighten, extend, and slip past one another, they assume in many cases new positions of entanglement with each other and with the fusible fibers, thus stabilizing the fabric and providing capacity for further extension before break.

Even though my finished fabrics are usually prepared from highly oriented carded webs, they are usually substantially more balanced than the fused fiber webs of the prior art because the three-dimensional frictional interlocking and entanglement of the cotton fibers in situ tends to randomize the orientation of the fibers. Individual fibers are less likely to be displaced or removed from the structure by abrasive forces, and in a direction normal to the plane of the sheet material the entanglement of the fibers greatly enhances the resistance to delamination of my products, particularly in those instances in which they have been prepared from a plurality of carded webs.

Because of their substantial tensile strength and other characteristics, my products are useful in the medical and surgical field as sponges, dressing pads, bandages and the like. No separate fusing treatment may be required because the activation of some fusible fibers may be effected by standard heat sterilization procedures employed in the preparation of bandages and the like in hospitals. Many of the sheet materials of this invention, prior to substantial activation of the fusible fibers, have distinct advantages in the manufacture of shaped liner or covering materials, stiffeners, and stiffened shaped articles. Their conformability and extensibility enable them to be easily molded or drawn to the desired shape, and thereafter the fusible fibers may be activated by heat or the action of appropriate solvents, thereby stabilizing the material in its molded shape and producing a surface with a high resistance to deformation.

My novel sheet materials are particularly adapted for use in the manufacture of end products where both high marginal tear resistance and interior softness and absorbency are required, as for example sanitary napkins and diapers. In making such products, the sheet material may be cut to the desired shape and heat pressed at its edges 55 only, thereby activating the fusible fibers in these areas while leaving a soft, fluffy absorbent interior region.

The fusible fibers contained in my structures may be selected from a very wide variety of materials. For example, various fibers comprising esters and ethers of cellulose are suitable, such as those made of cellulose acetate, cellulose propionate, cellulose butyrate, ethyl cellulose and benzyl cellulose. Fibers made of mixed esters such as cellulose acetate-propionate also are very useful. Others of an entirely different chemical nature, however, 60 may be employed, such as those made of vinyl polymers, for example, polyvinyl chloride, polyvinyl acetate, polyvinylidene chloride, or vinyl copolymers, and those of the polyamide type, an important example of which is that commercially known as nylon. The above mentioned fusible fibers may be classified as thermosensitive, that is, they have the property of being softened by heat and hardening upon cooling again, although they may be also

rendered tacky by the use of appropriate organic solvents. Under certain conditions, to be described hereinafter, I may also use fibers which are not classified as thermosensitive.

I have found that the felt-like sheet materials of this invention can be produced by mixing the cotton fibers with fibers having latent coalescent properties to form a web and subjecting the web or a plurality of such webs to treatment with alkaline liquids having a substantial swelling action on cellulose in such a manner as to permit shrinkage of the structure, these steps of the process and an apparatus useful in carrying these out being more fully disclosed in my copending application, Serial No. 643,799, filed January 26, 1946, now U. S. Patent No. 2,528,793, of which this application is a continuation-in-part. The assembly is then washed to remove the swelling agent and dried. Depending on their nature the fusible fibers may be activated by the alkaline treatment, by the heat employed in the drying process, by subsequent heat treatment or by the action of appropriate solvents or by suitable combinations thereof. Pressure may be used to increase the bonding by the activated fibers. The preferred treating chemical for the cotton fibers is an aqueous solution of caustic alkali such as sodium, potassium or lithium hydroxide, but other basic cellulose swelling agents may be employed, such as solutions of sodium zincate, quaternary ammonium bases such as benzyl trimethyl ammonium hydroxide and the like.

Using aqueous sodium hydroxide solutions satisfactory results have been obtained with solution concentrations of at least 8% and less than 30% NaOH at temperatures from just above the freezing point of the solution to +25° C. It should be understood that temperature and concentration are mutually dependent variables and that the selection of a particular value for one may fix the operating range of the other. Preferably and for best results such solutions are used in concentration of at least 10% and less than 18% NaOH at temperatures from -10° C. to +15° C. Other reagents may be employed at corresponding effective strength and temperature.

The maximum felting, contractive effects of the chemical are realized in a short time, normally in 1/2 to 3 minutes and the fiber sheet is then removed from the vat and treated to remove the chemical; preferably promptly as over long exposure to the chemical may produce undesirable gelatinization of the fibers.

The extent of fiber curling, kinking, and entanglement in situ, after the mixing and sheeting of the two classes of the fibers, and upon which the unique features of this invention are dependent, is indicated roughly by the permanent area contraction of my sheet materials during the first stage of my process. I have found that the most satisfactory results have been obtained when this contraction is of the order of 30 percent or greater, although products whose area shrinkages are less may possess some or many of the features of this invention.

The amount of shrinkage obtained depends on a number of factors, the most important of which are the weight per unit area of the fibrous assembly to be treated, the ratio by weight of the cotton fibers to the fusible fibers, and the temperature and concentration of the caustic solution. Other things being equal, the area shrinkages decrease if either the weight of the assembly or the relative proportion of fusible fibers to cotton fibers is increased. For most products of this invention, the cotton fibers should be in major proportion in order to have the greatest flexibility of operating conditions, although satisfactory shrinkages have been observed with cotton fiber concentrations somewhat lower than 50 percent in conjunction with optimum values of the other factors influencing area contraction of the assembly.

In my preferred material the fusible fibers are thermoplastic in character and substantially inert to my alkaline treating agent under the temperature, concentration, and time duration condition of my process. The duration of

contact of the fusible fibers with the treating solution is particularly important in the case of thermoplastic fibers of a cellulosic nature such as cellulose acetate where prolonged contact might radically change the characteristics of the fibers, reducing or destroying their thermoplastic properties. Also, fibers of this type may in some instances be rendered coalescent in the caustic solution, depending on the particular fiber and conditions of treatment, causing bonding of the fibers prior to heat or solvent activation. Usually, however, the bonding supplied by the fusible fibers as a result of the caustic-treating stage of my process is only incidental, and the fusible fibers retain their latent coalescent properties to a substantial extent.

The particular type of thermoplastic fiber chosen depends primarily on the character of the product desired. In order to produce a fluffy, highly extensible structure the fusible fibers of which are to be activated at some point in the end use of the material, I select a fusible fiber which becomes tacky and coalescent at a relatively high temperature so as to minimize the activation of the fusible fibers in the drying of the sheet material following caustic treatment. It is possible, of course, to achieve these same results with fibers which become tacky at lower temperatures by reducing the drying temperature, but this is inefficient from an operating viewpoint. Conversely, if a product is desired in which the fusible fibers are partially or completely activated, the drying temperature may be increased, or a fusible fiber may be selected which becomes tacky and coalescent at a relatively low temperature.

The operation of activating the fusible fibers should be controlled in accordance with the nature of the binder fibers used, the proportion of such fibers, and the characteristics of the final product desired. During the mixing step these fibers can be in a dry free condition suitable for dry assembly, picking, carding or like processes. Consequently, the process of activation necessarily requires that the binder fibers be softened to a suitable degree. Any appropriate activating agent may be used which will produce good softening action. Those found most practical consist of heat, solvents or those substances such as plasticizers which exert a softening action, or some combination of the foregoing. Where the binder fibers are thermosensitive, having the property of being softened by heat and hardening upon cooling again, these changes in the physical condition ordinarily take place without any material chemical deterioration. Accordingly, a convenient method of effecting activation is to pass the sheet material through a heating chamber, between heated plates or heated rolls, or through any other suitable apparatus, such as a dielectric heating unit, capable of raising the temperature of the fibers to the desired degree.

Where the binder fibers used are soluble in or may be softened by organic solvents which do not affect the cotton fibers to any substantial degree, another method of producing the desired union of the fibers consists in subjecting the material after caustic treatment to the action of such a solvent, or to a solvent vapor or gas, which will develop in situ the adhesive or bonding properties of the fusible fibers. For instance, if the sheet material consists of a mixture of cotton and cellulose acetate fibers it may be treated with a mixture of acetone and methanol to superficially dissolve or soften the fusible fibers. The web may then be passed between pressure rolls. The nature of the solvents employed necessarily will be determined by the character of the binder fibers and other practical considerations. A wide variety of solvents for the various binder fibers above mentioned are known, including acetone, methyl alcohol, monomethyl ether of ethylene glycol, propylene oxide, methyl acetate, acetic acid, diacetone, chlorobenzene, dimethyl formamide, chloroform, toluene, and diethyl ether, the particular solvent chosen depending on the chemical composition of the binder fiber employed.

Whether or not pressure be used in the activation

process will depend chiefly upon the nature of the fusible fibers used and of the character of the final product desired. Pressing necessarily results in bringing a single fusible fiber in contact with a greater number of contiguous fibers of both kinds than otherwise would be the case and thus to increase the number of individual bonds with accompanying increase in strength. It tends to reduce the softness, flexibility and draping qualities of the product and to give it greater firmness and rigidity. Whether to use pressure and the degree of pressure to be employed, if it is used, therefore will depend upon results desired, the nature of the fusible fiber and softening agent used and other practical considerations.

That the nature of the bonding, coalescence or association of the fibers with each other produced by the activation process may take several forms will be evident from the character of the activation processes herein described. For example, in subjecting the sheet material to a suitable temperature the thermoplastic fibers will attain a softening stage which is sufficient to develop the coalescent properties. Or with some types of binder fibers, the heating step may be carried further until the surfaces of the fiber become sticky so that when the web is pressed the binder fibers will adhere or weld firmly to other binder fibers, and they likewise adhere to the non-binder fibers with which they are in contact. Or with some kinds of fusible fibers the heating step may be continued still further until the form of the binder is further broken down and the fibers are converted into almost a liquid state in which case they will wet intersecting non-binder fibers and will unite them upon subsequent cooling. In any of these extremely soft conditions more or less spreading the binder constituent may be effected, if desired, and even to such a point as to convert some or almost all of the fusible fibers into discreet particles or a discontinuous or continuous non-fibrous film.

In those instances where heat is employed as an activating agent for the fusible fibers it is possible to obtain more uniform bonding action throughout the sheet material by matching the thermo-softening point of the fusible fibers to the temperature gradient throughout the thickness of the web. This matching may be accomplished by incorporating different amounts of plasticizer into fusible fibers in the various strata of the sheet material or by selecting chemically different fusible fibers with varying softening temperatures.

When my products are prepared with a relatively high proportion of thermoplastic fibers at at least one surface of the material, they are useful for purposes to which heat sealability is desired, as for example, in porous or permeable containers. Sheet materials which exhibit different surface characteristics because the fusible fibers occur in predetermined different proportions on opposite surfaces are particularly useful as adhesive tape backings because good interface adhesion and resistance to picking on unrolling are secured.

By incorporating yarns or woven fabrics into my structures prior to caustic treatment it is possible to manufacture products similar to those described in my copending application S. N. 191,933, filed October 24, 1950. In these products the positive adhesive bonding supplied by the fusible fibers considerably strengthens the frictional entanglement of the spun and upspun fibers.

A class of fusible fibers may be used which are not thermosensitive but which swell and become gelatinous and tacky in the presence of the alkaline treating agents of my process. Examples of this class are fibers of regenerated cellulose manufactured according to the viscose or cuprammonium processes. One advantage inherent in the use of this class of fibers is that no after-treatment of the material is required. The cotton fibers are curled and kinked and the fusible fibers activated by the same treating solution. The extent of activation of this type of fusible fiber may be controlled by varying the temperature and concentration of the caustic, or by adding

5 varying amounts of sodium chloride to the wash water, or to the caustic. Products of this type have a high degree of stability, because the adhesive bonding provided by the regenerated cellulose fibers is substantially unaffected by heat or the action of a wide variety of organic solvents.

10 The following examples are given as illustrative of the products of my invention:

#### Example 1

Nineteen parts by weight of bleached cotton fibers were mixed in a picker lapper with one part Vynon fibers VYHH-2 (a co-polymer of vinyl acetate and vinyl chloride distributed by The American Viscose Company). The lap was fed to a card which carded the fiber mixture and worked it into the form of a web. Several such webs were superposed to form a fibrous sheet weighing approximately 70 grams per square yard. The fibrous sheet was cold-pressed by passing it between calender rolls at a pressure of about 1000 pounds per inch of roller inch of roller width and then treated in a bath of 14% NaOH at a temperature of  $-4^{\circ}$  C. for a period of about 35 seconds. The material was removed from the bath, rinsed with water, neutralized with dilute acetic acid, again washed, and dried in air. An area shrink of 77% was noted. Half of each sample was fused between layers of cheesecloth at  $300^{\circ}$  F., for five minutes without pressure and the following physical properties determined.

#### CORRECTED STRENGTH<sup>1</sup>

|                                     | Unfused |      | Fused |      |
|-------------------------------------|---------|------|-------|------|
|                                     | Dry     | Wet  | Dry   | Wet  |
| Lengthwise (machine direction)..... | 7.10    | 2.36 | 7.02  | 3.38 |
| Widthwise.....                      | 2.45    | .944 | 2.36  | 1.27 |
| Ratio (Lengthwise to Widthwise).... | 2.90    | 2.51 | 2.97  | 2.66 |

#### ELONGATION, PERCENT

|                 |     |     |    |     |
|-----------------|-----|-----|----|-----|
| Lengthwise..... | 89  | 110 | 88 | 93  |
| Widthwise.....  | 112 | 135 | 94 | 110 |

<sup>1</sup> Corrected strength: In making comparisons between felts of different thicknesses and densities I make use of what I term "corrected strength," which is the actual load at break (in pounds per inch of width of the sample tested) divided by the weight in pounds of one square yard of the felt. This corrected load takes into account differences in weight of the compared felts, in effect, giving the approximate strength of a unit quantity or weight of fibers on different felts.

#### Example 2

A fibrous sheet material containing 10% by weight Vynon fibers and 90% cotton fibers was prepared, treated, and tested as in Example 1. The area contraction was 66%.

#### CORRECTED STRENGTH

|                                     | Unfused |      | Fused |      |
|-------------------------------------|---------|------|-------|------|
|                                     | Dry     | Wet  | Dry   | Wet  |
| Lengthwise.....                     | 7.07    | 2.52 | 9.60  | 4.24 |
| Widthwise.....                      | 1.83    | .970 | 2.96  | 1.55 |
| Ratio (Lengthwise to Widthwise).... | 3.86    | 2.60 | 3.24  | 2.74 |

#### ELONGATION, PERCENT

|                 |    |     |    |    |
|-----------------|----|-----|----|----|
| Lengthwise..... | 55 | 71  | 56 | 64 |
| Widthwise.....  | 91 | 138 | 94 | 99 |

#### Example 3

A fibrous sheet material containing 20% by weight Vynon fibers and 80% cotton fibers was prepared,

7 treated and tested as in Example 1. The area contraction was 51%.

## CORRECTED STRENGTH

|                                 | Unfused |      | Fused |      |
|---------------------------------|---------|------|-------|------|
|                                 | Dry     | Wet  | Dry   | Wet  |
| Lengthwise                      | 7.02    | 3.24 | 17.8  | 10.2 |
| Widthwise                       | 1.81    | .666 | 4.53  | 2.70 |
| Ratio (Lengthwise to Widthwise) | 3.93    | 4.97 | 3.94  | 3.78 |
| ELONGATION, PERCENT             |         |      |       |      |
| Lengthwise                      | 33      | 48   | 37    | 43   |
| Widthwise                       | 106     | 114  | 77    | 44   |

## Example 4

A fibrous sheet material containing 40% by weight Vinyon fibers and 60% cotton fibers was prepared, treated and tested as in Example 1. The area contraction was 31%.

## CORRECTED STRENGTH

|                                 | Unfused |      | Fused |      |
|---------------------------------|---------|------|-------|------|
|                                 | Dry     | Wet  | Dry   | Wet  |
| Lengthwise                      | 4.71    | 2.49 | 29.9  | 17.7 |
| Widthwise                       | 1.64    | .853 | 8.03  | 4.72 |
| Ratio (Lengthwise to Widthwise) | 2.87    | 2.92 | 3.72  | 3.75 |
| ELONGATION, PERCENT             |         |      |       |      |
| Lengthwise                      | 26      | 37   | 25    | 33   |
| Widthwise                       | 83      | 131  | 57    | 42   |

## Example 5

A fibrous sheet weighing 60 grams per square yard containing 10% by weight Vinyon fibers and 90% cotton fibers was prepared and treated as in Example 1 except that nip rolls at a pressure of about ten pounds per inch of roller width were substituted for the heavy calender rolls. The area contraction of the air-dried material was 72.6%. The following physical properties were determined:

## Corrected strength

|            |      |
|------------|------|
| Lengthwise | 8.48 |
| Widthwise  | 2.36 |
| Ratio      | 3.59 |
| Lengthwise | 55.7 |
| Widthwise  | 70.4 |

## Example 6

A 10% Vinyon-90% cotton fibrous sheet weighing 30 grams per square yard was prepared according to the method of Example 1 and given a light press by passing it through nip rolls at a pressure of about ten pounds per inch of roller width. The sheet was then treated in a bath of 18.4% NaOH at 10° C., washed with water, neutralized with dilute acetic acid, and again washed with water. An area contraction of about 38% was observed. A portion of the material was air-dried and the remainder dried on a steam can maintained at about 225° F. Part of the can-dried portion was subjected for a period of one minute to a pressure of 386 pounds per square inch be-

tween metal plates heated to 295° F. The following physical properties of each material were determined:

## CORRECTED STRENGTH

|            | CORRECTED STRENGTH |           |             |
|------------|--------------------|-----------|-------------|
|            | Air Dried          | Can Dried | Hot Pressed |
| Lengthwise | 11.6               | 10.8      | 41.2        |
| Widthwise  | 1.10               | 1.13      | 6.09        |
| Ratio      | 10.5               | 9.58      | 6.76        |

## ELONGATION, PERCENT

|            |      |      |      |
|------------|------|------|------|
| Lengthwise | 20.9 | 20.9 | 13.9 |
| Widthwise  | 44.1 | 72.4 | 6.2  |

## Example 7

A 40% Vinyon, 60% cotton fibrous sheet weighing 108 grams per square yard was prepared according to the method of Example 1 and given a light press by passing it through nip rolls at a pressure of about ten pounds per inch of roller width. The sheet was then treated in a bath of 13.8% NaOH at 4° C., washed with water, neutralized with dilute acetic acid, and again washed with water. An area shrink of 62.5% was noted. A portion of the material was air dried and the remainder dried on a steam can at a temperature of about 225° F. Part of the can-dried portion was subjected for a period of one minute to a pressure of 22.1 pounds per square inch between metal plates heated to 290° F. The following physical properties of each material were determined:

## CORRECTED STRENGTH

|            | CORRECTED STRENGTH |           |             |
|------------|--------------------|-----------|-------------|
|            | Air Dried          | Can Dried | Hot Pressed |
| Lengthwise | 8.60               | 15.6      | 75.4        |
| Widthwise  | 1.40               | 1.55      | 8.70        |
| Ratio      | 6.15               | 10.1      | 8.65        |

## ELONGATION, PERCENT

|            |      |      |      |
|------------|------|------|------|
| Lengthwise | 10.2 | 9.0  | 16.0 |
| Widthwise  | 62.7 | 47.4 | 7.6  |

## Example 8

A fibrous sheet weighing 44 grams per square yard consisting of 80% bleached cotton fibers and 20 percent fusible fibers composed of two parts cellulose acetate and one part paratoluene ethyl sulfonamide was prepared according to the method of Example 1 and given a light press by passing it through nip rolls at a pressure of about ten pounds per inch of roller width. The sheet was then treated in a bath of 11.7% NaOH at -2° C., washed with water, neutralized with dilute acetic acid, and again washed with water. An area shrink of 62.3% was observed. A portion of the material was air dried and the remainder dried on a steam can maintained at about 225° F. Part of the can-dried portion was sprayed with acetone, pressed with a cardboard roller under hand pressure and dried on the steam can. The product was noticeably stiffer and stronger than either of the other samples. The following physical properties of each material were determined:

## CORRECTED STRENGTH

|            | CORRECTED STRENGTH |           |               |
|------------|--------------------|-----------|---------------|
|            | Air-Dried          | Can-Dried | Solvent-Fused |
| Lengthwise | 11.0               | 8.7       | 19.3          |
| Widthwise  | 2.12               | 3.48      | 9.25          |
| Ratio      | 5.2                | 2.50      | 2.09          |

## ELONGATION, PERCENT

|            |      |      |      |
|------------|------|------|------|
| Lengthwise | 17.4 | 18.9 | 11.4 |
| Widthwise  | 29.1 | 10.1 | 11.6 |

## Example 9

A fibrous sheet weighing 94.5 grams per square yard consisting of 60% cotton fibers and 40% viscose rayon fibers was prepared according to the method of Example 1 and given a light press by passing it through nip rolls at a pressure of about ten pounds per inch of roller width. The sheet was then treated in a bath of 20% NaOH at 21° C., washed with water containing 10% sodium chloride, neutralized with dilute acetic acid, again washed with water and dried on a steam can. An area contraction of approximately 30% was observed. The following physical properties were determined:

|            | Corrected strength  |
|------------|---------------------|
| Lengthwise | 2.97                |
| Widthwise  | .420                |
| Ratio      | 7.08                |
|            | 15                  |
|            | Elongation, percent |
| Lengthwise | 24.6                |
| Widthwise  | 122.6               |
|            | 20                  |

## Example 10

A fibrous sheet weighing approximately 91 grams per square yard consisting of 60% cotton fibers and 40% viscose rayon fibers was prepared according to the method of Example 1 and given a light press by passing it through nip rolls at a pressure of about ten pounds per inch of roller width. The sheet was then treated in a bath of 20% NaOH at 21° C., washed with water, neutralized with dilute acetic acid, again washed with water and dried on a steam can. An area contraction of 56% was noted. The following physical properties of the material were observed.

|            | Corrected strength  |
|------------|---------------------|
| Lengthwise | 14.0                |
| Widthwise  | 4.76                |
| Ratio      | 2.94                |
|            | 30                  |
|            | Elongation, percent |
| Lengthwise | 14.5                |
| Widthwise  | 6.95                |
|            | 35                  |
|            | 40                  |

## I claim:

As an article of manufacture, a unitile, coherent, integrated, shrunken textile sheet material having substantial extensibility, conformability, integrity, and resilience and consisting essentially of fibers having latent coalescent properties and unspun cotton fibers, said unspun cotton fibers being chemically swollen, said fibers having latent coalescent properties and said unspun cotton fibers being mutually integrated and frictionally interlocked by chemically induced permanent deformations of said unspun cotton fibers, said deformations being in the form of random kinks, bends, twists, and curls in substantially all three-dimensional directions and being in excess of the deformations normally present in cotton fibers, the unspun cotton fibers being entangled with themselves and with each other and with said fibers having latent coalescent properties, the entanglement being substantially continuous and uniform throughout the sheet, said fibers having latent coalescent properties being adhesively bonded at some at least of their points of contact with each other and with said cotton fibers by the activation of their coalescent properties.

## References Cited in the file of this patent

## UNITED STATES PATENTS

|           |              |       |               |
|-----------|--------------|-------|---------------|
| 2,181,043 | Boeddinghaus | ----- | Nov. 27, 1939 |
| 2,277,049 | Reed         | ----- | Mar. 24, 1942 |
| 2,321,108 | Schneider    | ----- | June 8, 1943  |
| 2,336,797 | Maxwell      | ----- | Dec. 14, 1943 |
| 2,348,079 | Lichtenthal  | ----- | May 2, 1944   |
| 2,395,371 | Dockerty     | ----- | Feb. 19, 1946 |
| 2,496,873 | Hoffman      | ----- | Feb. 7, 1950  |
| 2,528,793 | Secrist      | ----- | Nov. 7, 1950  |